

## 1

2,816,028

## POLYMERIC GENTISAMIDE ANTISTAIN AGENTS FOR COLOR PHOTOGRAPHY

Louis M. Minsk, Rochester, N. Y., assignor to Eastman Kodak Company, Rochester, N. Y., a corporation of New Jersey

No Drawing. Application July 29, 1955,  
Serial No. 525,366

6 Claims. (Cl. 96—100)

This invention relates to color photography and particularly to a method for preventing the formation of color fog or stain in photographic emulsions.

The method of color photography in which color-forming or coupler compounds combine with the development product of aromatic amino photographic developers to produce dyes is well known. The color formers or couplers may be added directly to the emulsion layers or may be incorporated in the developing solution as described in Fischer U. S. Patent 1,102,028, granted June 30, 1914, or they may be incorporated in a water-permeable medium which is insoluble in the carrier for the sensitive silver salt as described in Mannes & Godowsky U. S. Patent 2,304,940, December 15, 1942, and Jelley and Vittum U. S. Patent 2,322,027, granted June 15, 1943.

A difficulty frequently encountered in these processes is the formation of color fog or stain. When the exposed



material is developed in a color forming developer, dye fog is frequently formed in the emulsion layer. This is because the developing agent has been oxidized to some extent by the action of the air and the oxidized developer tends to couple with the color-forming compound at places in the photographic material where no silver image is produced. It is well known that in these processes the dye should be formed only where the silver halide is reduced to metallic silver, thereby oxidizing the developing agent to a form which couples with the color former. Once the developing agent is oxidized, it couples immediately with the color former whether a photographic image is present or not. Aerial oxidation of the developer or oxidation by means other than development of the photographic image therefore converts the developer to a form which will immediately react with the color



former to produce a color fog or stain. This effect is especially noticeable in materials having couplers incorporated in the sensitive emulsion layer since there is no coupler in the developing solution to react with any

developing agent which is oxidized by the action of the air. Fog or stain arising from these causes is not readily controlled by the same procedures used to control silver fog.

5 The incorporation of various compounds in photographic emulsions for controlling color fog or stain has been described in Weissberger and Vittum U. S. Patent 2,356,486, August 22, 1944, and Vittum and Wilder U. S. Patent 2,360,290, October 10, 1944. However, the 10 use of these simple reducing agents for preventing or controlling color fog or stain has a distinct disadvantage in that they have a tendency to wander from the areas in which they have been placed into other areas of the photographic composition where they have harmful effects. In certain color processes the compounds are placed in the area of the emulsion containing the coupler and act on it to produce undesired effects.

15 It is, therefore, an object of the present invention to provide a novel means for reducing or eliminating the 20 formation of color fog or stain in photographic emulsions. A further object is to provide suitable non-diffusing reducing agents for incorporation in color photographic materials. A further object is to provide a color forming photographic emulsion having non-diffusing couplers 25 and non-diffusing stain or fog inhibitors incorporated therein. Other objects will appear from the following description of my invention.

These objects are accomplished by incorporating in a silver halide emulsion containing color couplers, a non-diffusing polymeric compound having the structure



in which A is hydrogen, an alkyl radical, e. g., methyl or ethyl, or a halogen atom, e. g., chlorine, B is hydrogen or an alkyl radical, e. g., methyl or ethyl, Z is an oxygen atom or —NH—, n is a positive integer of 1 to 6, and x and y are positive integers, for example, from 50 to 2000.

45 Instead of the styrene unit, the polymer may have a vinyl butyl ether unit or an acrylic acid unit, as illustrated below.

The antistain agents which I propose to use are prepared by the reaction of a styrene-maleic anhydride intermediate and a derivative of gentisamide. The preparation of the styrene-maleic anhydride intermediate is described in Godowsky U. S. Patent 2,698,794.

The following compounds are suitable for use according to my invention.



This compound was prepared by the reaction of a styrene-maleic anhydride intermediate and N-β-hydroxyethylgentisamide. In the preparation, water is ultimately added to open any residual anhydride.



This compound was prepared by the reaction of a styrene-maleic anhydride intermediate with N- $\beta$ -aminoethylgentisamide.

(3)



This compound was prepared by the reaction of a vinyl butyl ether-maleic anhydride interpolymer with N- $\beta$ -aminoethylgentisamide.

bility of the coupler in the emulsion, either to heat or to visible or ultraviolet radiation should not be decreased by added agents and it is found that my compounds are



helpful in this respect also. In mixed packet systems it is also desirable to improve color separation between the packets and my compounds are of use for this purpose.

(4)



This compound was prepared by the reaction of a vinyl toluene-maleic anhydride interpolymer with N- $\beta$ -aminoethylgentisamide.

(5) Reaction product of styrene-itaconic anhydride interpolymer and N- $\beta$ -aminoethylgentisamide.

(6) Reaction product of dichlorostyrene-maleic anhydride interpolymer and N- $\beta$ -aminoethylgentisamide.

(7) Reaction product of styrene-citraconic anhydride interpolymer and N- $\beta$ -aminoethylgentisamide.

The following examples illustrate the way in which my compounds may be used.

## EXAMPLE 1

This example shows the improvement in stain and "print-out" achieved by the use of my compounds. Stain was measured by determining at various wave-lengths the reflectance of an unexposed, processed emulsion coated 25 on a reflecting cellulosic support. Comparison of this re-

(8)



This compound was prepared by the reaction of polyacrylic anhydride and N- $\beta$ -aminoethylgentisamide.

(9) Reaction product of styrene-maleic anhydride interpolymer and N- $\beta$ -hydroxyethylhomogentisamide.

(10) Reaction product of styrene-maleic anhydride interpolymer and N- $\gamma$ -aminopropylgentisamide.

My compounds are useful in silver halide emulsions containing color couplers of the type which couple with the oxidation product of primary aromatic amino developing agents. My compounds can be used in emulsions of the type in which the coupler is incorporated directly in the gelatin in the form of a water-soluble but non-diffusing compound or in which the coupler is dissolved in an organic solvent before dispersion in the emulsion as described in Jelley and Vittum U. S. Patent 2,322,027, or in mixed packet systems of the type described in Godowsky U. S. Patent 2,698,794. My compounds are usually employed in amounts ranging from 0.5% to 20% of the amount of coupler used in the emulsion although more or less of the polymeric anti-stain agent may be employed as desired or necessary. My compounds have the capacity to form packets, and when used in the Godowsky system probably occur in the packet phase.

My agents may be used to improve various properties of photographic emulsions containing couplers. Stain in the emulsion due to the reaction between coupler and oxidized developer formed either by aerial oxidation or by the processing solutions may be reduced in certain cases by the use of my compounds. Stability of the dye resulting from color development should not be impaired by agents added to the emulsion and experiments show that my compounds are satisfactory in this respect. Sta-

50 flectance with that obtained for uncoated support indicated the effectiveness of the agent being tested, the results being expressed as a percentage of the reflectance of the uncoated support. "Print-out" or stability to visible and ultra-violet radiation, was measured as loss in percent transmittance of the unexposed processed sample before and after 6 hours exposure in the Fad-O-Meter.

55 A solution of 4 grams of the coupler 2-(2,5-diaminophenoxyacetamino)-4,6-dichloro-5-methylphenol and varying amounts of Compound 1 in 10 cc. of di-n-butylphthalate was prepared by heating a mixture of the components to 150° C. The hot solutions were each poured with stirring into 160 cc. of an aqueous solution of 30 cc. of 10% gelatin solution and 4 cc. of 5% alkanol B solution (sodium triisopropylnaphthalene sulfonate). The resulting mixtures were each recycled through a colloid mill for 5 minutes, and the resulting fine dispersions were each mixed with 100 grams of a melted gelatin-silver bromide emulsion. The mixtures were then coated on white pigmented film support and dried. After exposure to a density scale and processing in a diethyl-p-phenylenediamine developer, the samples were fixed and stain and print-out were determined as indicated above, with the following results:

| Compound 1, gram per sq. ft. | Stain, Reflectance at 670 m $\mu$ | Print-out Reflectance |
|------------------------------|-----------------------------------|-----------------------|
|                              | Percent                           | Percent               |
| 0                            | 71                                | 10.5                  |
| .02                          | 82                                | 8                     |
| .05                          | 82                                | 5.5                   |
| .10                          | 81.5                              | 1.0                   |
| .15                          | 80                                | 0                     |

Increasing stain reflectance indicates a reduction in stain, and decreasing print-out reflectance indicates a decrease in print-out, as the concentration of antistain agent is increased.

## EXAMPLE 2

This example was the same as Example 1 except that instead of the cyan coupler of Example 1 there was used 4 grams of the coupler N-(4-benzoylacetaminobenzenesulfonyl)-N-( $\gamma$ -phenylpropyl)-p-toluidine. After processing the unexposed coating as in Example 1, stain and print-out were determined as in Example 1 with the following results:

| Compound 1, gram per sq. ft. | Stain, Reflectance at 440 m $\mu$ |         | Print-out, Reflectance |         |
|------------------------------|-----------------------------------|---------|------------------------|---------|
|                              | Percent                           | Percent | Percent                | Percent |
| 0.....                       | 76                                | 26.5    |                        |         |
| .02.....                     | 73.5                              | 19.5    |                        |         |
| .05.....                     | 69                                | 13      |                        |         |
| .10.....                     | 63.5                              | 6.5     |                        |         |
| .15.....                     | 62.6                              | 6       |                        |         |

## EXAMPLE 3

Separate emulsion coatings were made as in Example 1, using 1, 5 and 25 mg. per sq. ft. of compounds 3 to 10. After exposure to a density scale and processing in a diethyl-p-phenylenediamine developer, the samples were fixed, and the amount of stain in the unexposed regions, and the amount of dye loss, were determined. To determine stain, the cyan dye density in unexposed regions was read through a Wratten No. 25 filter, before and after exposure for 6 hours in a Fade-O-Meter. Cyan dye loss was determined by reading the cyan dye density before and after exposure in the Fade-O-Meter, and calculating the percentage loss. For comparison purposes, samples containing no anti-stain agent, and containing 1 and 5 mgs. of 2,5-di-tert. octyl hydroquinone, were treated in the same way. The results were as follows:

| Sample                | Stain |           | Cyan dye loss<br>(Six-hour<br>Fade-O-<br>Meter) |
|-----------------------|-------|-----------|-------------------------------------------------|
|                       | Fresh | Incubated |                                                 |
| None.....             | .265  | .28       | 5.1                                             |
| Dioctyl hydroquinone: |       |           |                                                 |
| 1 mg.....             | .19   | .225      | 2.6                                             |
| 5 mg.....             | .195  | .19       | 9.5                                             |
| Compound 3:           |       |           |                                                 |
| 1 mg.....             | .205  | .25       | 2.7                                             |
| 5 mg.....             | .15   | .215      | 8.3                                             |
| 25 mg.....            | .125  | .145      | 5.4                                             |
| Compound 4:           |       |           |                                                 |
| 1 mg.....             | .22   | .305      | 4.9                                             |
| 5 mg.....             | .17   | .24       | 6.1                                             |
| 25 mg.....            | .145  | .175      | 5.4                                             |
| Compound 5:           |       |           |                                                 |
| 1 mg.....             | .245  | .315      | 2.9                                             |
| 5 mg.....             | .20   | .30       | 3.0                                             |
| 25 mg.....            | .165  | .21       | 4.1                                             |
| Compound 6:           |       |           |                                                 |
| 1 mg.....             | .28   | .34       | 5.8                                             |
| 5 mg.....             | .225  | .315      | 4.1                                             |
| 25 mg.....            | .165  | .24       | 4.9                                             |
| Compound 7:           |       |           |                                                 |
| 1 mg.....             | .245  | .295      | 4.2                                             |
| 5 mg.....             | .195  | .275      | 3.8                                             |
| 25 mg.....            | .15   | .215      | 3.7                                             |
| Compound 8:           |       |           |                                                 |
| 1 mg.....             | .18   | .23       | 4.3                                             |
| 5 mg.....             | .135  | .165      | 4.7                                             |
| 25 mg.....            | .11   | .12       | 2.6                                             |
| Compound 9:           |       |           |                                                 |
| 1 mg.....             | .28   | .325      | 5.1                                             |
| 5 mg.....             | .335  | .345      | 3.9                                             |
| 25 mg.....            | .19   | .215      | 3.2                                             |
| Compound 10:          |       |           |                                                 |
| 1 mg.....             | .21   | .265      | 5.7                                             |
| 5 mg.....             | .155  | .205      | 5.2                                             |
| 25 mg.....            | .125  | .155      | 2.5                                             |

## EXAMPLE 4

This example shows the improvement in stain and print-out achieved by the use of my compounds in a packet system.

A cyan coupler dispersion was made by dissolving 4.3 grams of the cyan coupler used in Example 1 in 5 cc. of n-butylphthalate at 150° C., adding the solution to 5 cc. of a 5% solution of alkanol B dispersing agent in 25 cc. of 5 10% gelatin solution and dispersing it therein.

Six grams of a red-sensitive gelatino-silver bromoiodide emulsion were added to 8 grams of the cyan coupler dispersion and mixed with a fast stirrer for 10 minutes. 10 Twelve cc. of a 10% solution of a copolymer of methacrylic acid and methyl- $\alpha$ -methacrylate (sodium salt) were mixed with 100 cc. of distilled water. The emulsion-coupler dispersion was added to the copolymer solution and this was stirred for 10 minutes more. To this mixture 15 was added a mixture of 4 cc. of a 2.5% solution of the ammonium salt of styrene-maleamic acid polymer and 4 cc. of a 2.5% solution of the sodium salt of compound 3 and the whole dispersion was stirred at 42° C. for one hour. Then 50 cc. of an 18% gelatin solution were added and mixed. The resulting packets contained 20 10 g. of compound 3 per mole of silver.

A similar emulsion was made without the antistain agent and both coatings were exposed and developed, and tested for cyan dye loss and stain as in Example 3. Results were as follows:

|                                   | Cyan dye loss<br>(6 Hour Fade-O-Meter) | Stain<br>(Fresh Test) |
|-----------------------------------|----------------------------------------|-----------------------|
| 30 Check coating.....             | None                                   | .09                   |
| Coating with antistain agent..... | None                                   | .01                   |

## EXAMPLE 5

This example shows the improvement in dye stability 35 achieved by the use of my compounds. Stability of the coupled dye to visible and ultra-violet radiation was determined by measuring the loss in density of the dye at its maximum spectral absorption, after exposure in the Fade-O-Meter for comparable periods of time, as in the preceding examples.

A dispersion of the cyan coupler of Example 1 was 40 made as described in Example 4, containing sufficient 2,5-di-tert.-octyl hydroquinone to give 0.5 mg. per square foot in the resulting coating. This dispersion was mixed with a red-sensitive gelatino-silver halide emulsion and packets 45 formed as described in Example 4. This coating was designated "A."

A similar dispersion was made without the dioctyl 50 hydroquinone and was mixed with a similar dispersion in equal amount, of an emulsion containing the magenta coupler 1-(p-tert. butylphenoxy)-phenyl-3- $\alpha$ -(p-tert. butylphenoxy propionylamino) - 5 - pyrazolone. This mixed emulsion was coated and designated "B."

A mixed emulsion of cyan and magenta coupler similar 55 to B was made but containing in the cyan packets sufficient 2,5-di-tert. octyl hydroquinone to give 50 mgs. per square foot in the resulting coating. This mixed emulsion was coated and designated "C."

A mixed cyan and magenta packet coating similar to C 60 was made but containing instead of the dioctyl hydroquinone, sufficient styrene-maleic acid-gentisamide anti-stain agent (compound 1) to give 14 mgs. per square foot of the resulting coating. This mixed emulsion was coated and designated "D."

Each of the coatings were exposed on an Eastman type 65 Ib Sensitometer and was then developed for 10 minutes at 68° F. in the following developing solution:

|                                    | Grams |
|------------------------------------|-------|
| 2-amino-5-diethylaminotoluene, HCl | 2     |
| Sodium sulfite                     | 2     |
| Sodium carbonate, monohydrate      | 20    |
| Potassium bromide                  | 2     |
| Water to 1 liter.                  |       |

After fixing, washing and bleaching each of the coatings 75 to remove residual silver and silver halide the coat-

ings were exposed for 6 hours on the Fade-O-Meter. Density readings were then taken at equivalent points in the exposure scale and were compared with readings of the same point in the scale before the Fade-O-Meter exposure. These gave readings of the amount of fading of the cyan dye, the readings having been made at 670 millimicrons. The change in density of the dye was as follows:

| Coating | Agent                                     | Density Loss |
|---------|-------------------------------------------|--------------|
| A.....  | 0.5 mg./sq. ft. dioctyl hydroquinone..... | .14          |
| B.....  | None.....                                 | .04          |
| C.....  | 50 mg./sq. ft. dioctyl hydroquinone.....  | .18          |
| D.....  | 14 mg./sq. ft. Compound 1.....            | 0.04         |

The loss in density of the cyan dye is shown to be much less than when dioctylhydroquinone (a prior art antistain compound) is used in the coating and is slightly less than when no antistain agent at all is used in the coating. At the same time the color separation in a mixed packet system was found to be improved by the use of my compound.

The compounds of my invention were prepared as follows:

*Compound 1.—Styrene-maleic anhydride-N- $\beta$ -hydroxyethyl gentisamide*

In an all-glass reflux outfit equipped with a mechanical stirrer and calcium chloride tube to keep out moisture, 50 g. of styrene-maleic anhydride interpolymer was dissolved in 500 ml. of dry pyridine. When doping was complete, 55 g. of N- $\beta$ -hydroxyethylgentisamide was added and the reaction was heated on a steam bath with stirring for two hours. Twenty-five milliliters of water was then added and heating was continued for an additional hour. The dope was poured into 8 liters of ether, with stirring. The precipitate was allowed to settle, the supernatant was decanted and replaced by 3 liters of fresh ether. The soft precipitate turned friable. It was filtered onto a Büchner and given three extractions with 3-liter portions of fresh ether, mechanically stirring for at least one hour and filtering after each. The friable product was dried in a vacuum desiccator under a constantly applied water pump vacuum. The yield was 115 g.; the nitrogen content, 3.8%; the hydroquinone equivalent, 36.7% (see below).

*Compound 2.—Styrene-maleic anhydride-N- $\beta$ -aminoethyl gentisamide*

*A. THE PREPARATION OF N- $\beta$ -AMINOETHYL GENTISAMIDE*

With mechanical stirring, 168 g. of methyl gentisate was added to 800 ml. of ethylenediamine over a 15-minute period. The temperature of the reaction mixture rose spontaneously to about 60° C. Stirring was continued for 4 1/4 hours during which the reaction returned to room temperature. The excess ethylenediamine was removed under reduced pressure and the residue was boiled with a solution of 1 liter of benzene and 400 ml. of absolute ethyl alcohol. With stirring, the oily residue changed to a crystalline solid. The crystals were filtered onto a Büchner funnel, washed on the funnel with a solution of 500 ml. of benzene and 200 ml. of absolute ethyl alcohol, and dried in a vacuum desiccator over calcium chloride under a constantly applied water pump vacuum. The crude material was recrystallized from 60-40 ethyl alcohol-water and redried as above. The yield ranged between 121 and 126 g. The melting points of different batches ranged from 194.5 to 196° (with decomposition). The nitrogen content was theoretical.

*B. REACTION OF STYRENE-MALEIC ANHYDRIDE INTERPOLYMER AND N- $\beta$ -AMINOETHYLGENTISAMIDE*

Fifty grams of styrene-maleic anhydride interpolymer was dispersed in 500 ml. of dry pyridine at 50° C. under

dry nitrogen in an all-glass outfit equipped with mechanical stirrer, gas inlet, and reflux condenser protected from moisture by calcium chloride tube. To the dope was added 155 g. of N- $\beta$ -aminoethylgentisamide and the heating and stirring at 55° C. under dry nitrogen was continued for 4 1/3 hours, when 125 ml. of distilled water was added and the reaction was heated for an additional hour. The dope was then poured into a stirred solution of 5 gal. of distilled water and 750 ml. of concentrated hydrochloric acid. The precipitate was stirred until nicely friable and filtered onto a Büchner funnel. The product was washed on the funnel with distilled water and then stirred for 15 minutes in a container with two successive 10-liter portions of distilled water, filtered onto a funnel after each. Most of the water was removed by drying in a vacuum desiccator over calcium chloride under a constantly applied water pump vacuum. The damp material was dissolved in 700 ml. of absolute ethyl alcohol, 5 g. of zinc dust was added, and the solution was brought to a boil. Concentrated hydrochloric acid was added slowly until the evolution of hydrogen began (a 8 ml.), when 5 g. more of zinc dust was added, followed by 5 ml. of concentrated hydrochloric acid. The reaction was allowed to proceed until no further decolorization occurred. The dope was then filtered through paper and precipitated after dilution by absolute ethyl alcohol to a volume of 1 liter, by pouring into 10 liters of stirred distilled water. The precipitate was filtered, washed on the funnel with distilled water, and stirred for 30 minutes in a beaker with two 3-liter portions of distilled water, filtering after each. The product was dried in a vacuum desiccator over calcium chloride under a constantly applied water pump vacuum. The yield was 86 g.; N=6.2%; hydroquinone equivalent, 39.9%.

*Compound 3.—Butyl vinyl ether-maleic anhydride-N- $\beta$ -aminoethylgentisamide*

Ten grams of vinyl butyl ether-maleic anhydride interpolymer was dispersed at 50° C. under nitrogen in 100 ml. of dry pyridine in an all-glass reflux outfit equipped with a mechanical stirrer. A smooth, deep violet dope was obtained. Eleven grams of N- $\beta$ -aminoethylgentisamide was added and the reaction was maintained at 50° C. under nitrogen with continuous stirring for five hours. Twenty-five milliliters of distilled water was added and the reaction mixture was stirred for an additional hour at 50° C. The dope was then diluted with 25 ml. of acetone and was poured in a fine stream into a stirred solution of 150 ml. of concentrated hydrochloric acid in 3 liters of distilled water. The precipitate obtained was washed with distilled water until free from acid and dried in a vacuum desiccator under a constantly applied water pump vacuum. The dry material was dissolved in 250 ml. of 10:1 by volume absolute ethyl alcohol: distilled water and heated on a steam bath with mechanical stirring. To the hot stirred dope was added 10 g. of zinc dust, followed by 7 ml. of concentrated hydrochloric acid. With the evolution of hydrogen, the color of the dope was bleached to a light yellow. The dope was filtered by suction through paper covered by a layer of filter aid and precipitated in 3 liters of distilled water containing 75 ml. of concentrated hydrochloric acid. The product was washed free from acid with distilled water and dried as above. The yield was 15 g.; N=6.6%; hydroquinone equivalent, 34.5%.

*Compound 4.—Vinyltoluene-maleic anhydride-N- $\beta$ -aminoethylgentisamide*

The general conditions of reaction and proportions were similar to those for compound 3. Zinc reduction was not used. The dope was diluted with alcohol prior to dilution. The yield was 18 g. The product analyzed 6.7% nitrogen and had a hydroquinone equivalent of 37.3%.

*Compound 5.—Styrene-itaconic anhydride-N- $\beta$ -aminoethylgentisamide*

The procedure and proportions were similar to those used for the reaction with the vinyl butyl ether-maleic anhydride interpolymer (compound 3), except that the zinc reduction step was omitted. The yield was 16 g. The nitrogen content was 6.4% and the hydroquinone equivalent 39.0%.

*Compound 6.—Dichlorostyrene-maleic anhydride-N- $\beta$ -aminoethylgentisamide*

The procedure used was similar to that for the vinyl-toluene-maleic anhydride interpolymer reaction (compound 4), except that double quantities were used. The yield was 26 grams. The nitrogen content was 4.0% and the hydroquinone equivalent 21.5%.

*Compound 7.—Styrene-citraconic anhydride-N- $\beta$ -aminoethylgentisamide*

The reaction conditions and proportions used were similar to those used for the dichlorostyrene-maleic anhydride reaction (compound 6), except that the product was further purified by another reprecipitation from acetone into water and hydrochloric acid followed by washing acid-free. The yield was 32.5 g. The nitrogen content was 6.5% and the hydroquinone equivalent 32.9%.

*Compound 8.—Polyacrylic anhydride-N- $\beta$ -aminoethylgentisamide*

In an all-glass reflux outfit equipped with reflux and calcium chloride tube, a mechanical stirrer and a gas inlet, 10 g. of polyacrylic anhydride was dispersed under dry nitrogen at 50° C. in 100 ml. of dry pyridine. To the dope was added 18 g. of N- $\beta$ -aminoethyl gentisamide and the reaction was continued with stirring at 50° C. After 2 hours, an additional 50 ml. of pyridine, and, after 5½ hours, 25 ml. of distilled water were added and heating and stirring continued for another hour. The dope was diluted with 100 ml. of acetone and poured in a fine stream into 3 liters of distilled water containing 225 ml. of concentrated hydrochloric acid. The rubbery precipitate was kneaded with fresh distilled water and then redissolved in 250 ml. of acetone. It was reprecipitated in 3 liters of distilled water containing 75 ml. of concentrated hydrochloric acid, washed with fresh distilled water until free from chloride, and dried in a vacuum desiccator over calcium chloride under a constantly applied water pump vacuum. The material with drying became brittle and could be ground. The yield was 11.0 g. The nitrogen content was 7.8% and the hydroquinone equivalent was 46.8%.

*Compound 9.—Styrene-maleic anhydride-N- $\beta$ -hydroxyethylhomogentisamide*

**A. THE PREPARATION OF N- $\beta$ -HYDROXYETHYLHOMOGENTISAMIDE**

Thirty grams of homogentisic lactone was added portionwise to a solution of 13.2 g. of ethanolamine in 100 ml. of methyl alcohol. There was some spontaneous warming. The reaction mixture was left at room temperature for one day. The methanol was then distilled away and the residue was dissolved with warming in 75 ml. of distilled water. After being made acid to Congo red with hydrochloric acid, the solution was successively treated with decolorizing carbon (Norite), filtered, and boiled with zinc dust. This removed most of the color. The solution was again made acid with hydrochloric acid, chilled, and filtered to remove a small amount of homogentisic lactone which crystallized out. The filtrate was concentrated at room temperature by vacuum to a syrup, and chilled. A slurry of crystals formed. The crystals were filtered onto a Büchner funnel, washed with a small amount of cold water, and dried in vacuum. Upon recrystallization from 2:1 abso-

lute ethyl alcohol: ligroin and drying, the product melted at 117.5–118.5° C. The yield was 12 g.

*Analysis.*—Calculated for N- $\beta$ -hydroxyethylhomogentisamide ( $C_{10}H_{13}O_4N$ ): C, 56.9%; H, 6.2%; N, 6.6%. Found: C, 56.9%; H, 6.3%; N, 6.6%.

**B. REACTION OF STYRENE-MALEIC ANHYDRIDE INTERPOLYMER AND N- $\beta$ -HYDROXYETHYLHOMOGENTISAMIDE**

Five grams of styrene-maleic anhydride interpolymer was dispersed in 50 ml. of dry pyridine in an all-glass reflux outfit equipped with a mechanical stirrer and protected from moisture by a calcium chloride tube. To this was added, with stirring, 6.0 g. of N- $\beta$ -hydroxyethylhomogentisamide and the reaction mixture was heated on a steam bath for one hour. Two and one-half milliliters of distilled water was then added and heating and stirring was continued for another hour. The dope was then cooled, diluted with 130 ml. of acetone and poured into 1500 ml. of ether with stirring. The precipitate was thoroughly extracted with ether and dried in a vacuum desiccator under a constantly applied water pump vacuum. The yield was 8.4 g. The nitrogen content was 3.1% and the hydroquinone equivalent was 24.0%.

*Compound 10.—Styrene-maleic anhydride-N- $\gamma$ -aminopropylgentisamide*

**A. THE PREPARATION OF N- $\gamma$ -AMINOPROPYLHOMOGENTISAMIDE**

Ten grams of methyl gentisate was added to 45 g. of 1,3-diaminopropane. Some heat was evolved. The flask was tightly stoppered and left at room temperature for one hour, during which time the reaction mixture changed to a slurry of crystals. This was diluted with 75 ml. of 5:2 benzene:absolute ethyl alcohol. The crystals were washed on the funnel with benzene-absolute ethyl alcohol (5:2) and dried. The product was recrystallized first from ethylene glycol monomethyl ether and then from absolute ethyl alcohol and water (55:45). This yield was 7 g.; melting point 209–210° C. (decomp.).

*Analysis.*—Calculated for N- $\gamma$ -aminopropylgentisamide ( $C_{10}H_{14}O_3N_2$ ): C, 57.1%; H, 6.7%; N, 13.3%. Found: C, 56.8%; H, 7.0%; N, 13.4%.

**B. REACTION WITH STYRENE-MALEIC ANHYDRIDE INTERPOLYMER**

The procedure used was quite similar to that used for the reaction of styrene-maleic anhydride interpolymer and N- $\beta$ -aminoethylgentisamide. Five grams of styrene-maleic anhydride interpolymer was dispersed at 50° C. under nitrogen in 50 ml. of dry pyridine in an all-glass outfit equipped with reflux condenser and calcium chloride tube, mechanical stirrer and gas inlet. Six grams of N- $\gamma$ -aminopropylgentisamide was added and the reaction mixture was stirred for 3½ hours at 50° C. Two and one-half milliliters of distilled water was added and, after ¾ hour, additional warming and stirring, the dope was diluted with 50 ml. of acetone and poured into 1.5 l. of distilled water containing 75 ml. of concentrated hydrochloric acid. The precipitate was filtered onto a Büchner funnel, washed on the funnel with distilled water and stirred ten minutes each with two 750-ml. portions of distilled water, filtering after each. The product was dried in a vacuum desiccator over calcium chloride under a constantly applied water pump vacuum. The yield was 9.0 g. The nitrogen content was 6.2%; the hydroquinone equivalent was 39.2%.

My stain inhibitors are particularly useful with paper materials where it is important to reduce the minimum or fog densities. This applies both to negative developing paper and to reversal paper. My stain inhibitors may, of course, also be used with transparent materials.

I have described the preparation of my anti-stain agents from gentisamide derivatives such as N- $\beta$ -hydroxyethylgentisamide. Homogentisamide derivatives may also be used, such as N- $\beta$ -hydroxyethyl homogentisamide and N-

11

$\beta$ -aminoethyl homogentisamide, in the preparation of my compounds.

Vehicles other than gelatin may be used in the emulsions in which my antistain agents are incorporated, e. g., polyvinyl alcohol, casein and its derivatives, gelatin derivatives, water-permeable cellulose derivatives, polyacrylamides, polyvinyl acetals or mixtures of these with gelatin.

It will be understood that the examples and modifications disclosed herein are exemplary only and that my invention is to be taken as limited only by the scope of 10 the appended claims.



I claim:

1. A color-forming photographic emulsion having reduced fogging tendency, comprising a silver halide emulsion having incorporated therein a non-diffusing color coupler capable of reacting with the oxidation product of a primary aromatic amino developer to produce a dye and, as an inhibitor of color stain, a non-diffusing polymeric compound having the structure:



where A is selected from the class consisting of hydrogen, alkyl radicals, and halogen radicals, B is selected from the class consisting of hydrogen and alkyl radicals, Z is selected from the class consisting of  $-\text{O}-$  and  $-\text{NH}-$ , x and y are positive integers from 50 to 2000, and n is a positive integer from 1 to 6.

2. A color-forming photographic emulsion having reduced fogging tendency, comprising a silver halide emulsion having incorporated therein a non-diffusing color coupler capable of reacting with the oxidation product of a primary aromatic amino developer to produce a dye and, as an inhibitor of color stain, a non-diffusing polymeric compound having the structure:



where R is selected from the units consisting of



where x and y are positive integers from 50 to 2000.

4. A color-forming photographic emulsion having reduced fogging tendency, comprising a silver halide emulsion having incorporated therein a non-diffusing color coupler capable of reacting with the oxidation product of a primary aromatic amino developer to produce a dye and, as an inhibitor of color stain, a non-diffusing polymeric compound having the structure:



where x and y are positive integers from 50 to 2000.

6. A color-forming photographic emulsion having reduced fogging tendency, comprising a silver halide emulsion having incorporated therein a non-diffusing color coupler capable of reacting with the oxidation product of a primary aromatic amino developer to produce a dye and, as an inhibitor of color stain, a non-diffusing polymeric compound having the structure:



A is selected from the class consisting of hydrogen, alkyl



radicals and halogen radicals, B is selected from the

where x and y are positive integers from 50 to 2000.

13

6. A color-forming photographic emulsion having reduced fogging tendency, comprising a silver halide emulsion having incorporated therein a non-diffusing color

14

of a primary aromatic amino developer to produce a dye and, as an inhibitor of color stain, a non-diffusing polymeric compound having the structure:



coupler capable of reacting with the oxidation product where  $x$  and  $y$  are positive integers from 50 to 2000.

No references cited.

UNITED STATES PATENT OFFICE  
Certificate of Correction

Patent No. 2,816,028

December 10, 1957

Louis M. Minsk

It is hereby certified that error appears in the printed specification of the above numbered patent requiring correction and that the said Letters Patent should read as corrected below.

Column 8, line 4, for "155 g." read —55 g.—; line 21, for "(ca 8 ml.)" read —(ca 8 ml.)—; column 12, claim 5, for that portion of the formula reading



Signed and sealed this 11th day of March 1958.

[SEAL]

Attest:

KARL H. AXLINE,  
*Attesting Officer.*

ROBERT C. WATSON,  
*Commissioner of Patents.*